

Nov. 7, 1950

B. L. TRILICH

2,529,060

SELF-SEALING WRAPPING MATERIAL

Filed Nov. 7, 1949

2 Sheets-Sheet 1



Inventor  
Bertram L. Trilich  
By Fred Gerlach atty.

Nov. 7, 1950

B. L. TRILLICH  
SELF-SEALING WRAPPING MATERIAL

2,529,060

Filed Nov. 7, 1949

2 Sheets-Sheet 2



## UNITED STATES PATENT OFFICE

2,529,060

## SELF-SEALING WRAPPING MATERIAL

Bertram L. Trillich, Winnetka, Ill., assignor to  
The Munising Paper Company, Chicago, Ill., a  
corporation of Ohio

Application November 7, 1949, Serial No. 125,973

9 Claims. (Cl. 117—68.5)

1

This invention relates to a wrapping material especially adapted for wrapping small articles and more particularly to a quick-sealing, moisture-proof, wrapping paper for wrapping a comestible to maintain its moisture content. In its preferred aspects, the invention relates to a quick-sealing, moisture-vapor-proof wrapping paper.

This application is a continuation-in-part of my copending application, Serial No. 659,278, filed April 3, 1946, now abandoned.

The wrapping material of the present invention consists of a paper-thin flexible carrier sheet, preferably of paper, having a flexible coating of a moisture-proof material, preferably a moisture-vapor-proof material, on one side thereof and on the other side a flexible coating or film of a self-adhering material which is substantially dry to the touch and substantially non-tacky but which is cohesive even under light pressure, and yet which is for all practical purposes non-adhesive to any surface such as paper, Cellophane, wood, glass, metal, paint, rubber, etc., devoid of said material. The self-adhering materials which may be used in accordance with the present invention are known materials and are usually termed "cohesive, substantially non-adhesive" materials. For convenience, these materials will be similarly referred to herein. Any such self-adhering materials may be used in accordance with the present invention.

The combination of a flexible water-proof coating on one side of a flexible carrier sheet and of a cohesive, substantially non-adhesive coating or film on the other provides a wrapping material for foodstuffs having desired moisture-proof or moisture-vapor-proof properties and a versatility and ease of use not heretofore present in any of the prior art wrapping materials, insofar as I am aware. The wrapping material of the present invention may be manipulated readily in sealing relationship about foodstuffs or dishes or other articles containing the same without the aid of heat or other extraneous expedients which entail skill and are inconvenient for the user.

In its preferred aspects the wrapping material of the present invention consists of a flexible, calendered paper sheet, one surface of which is coated with a flexible film or coating of a wax and the other with a film or coating of a cohesive, substantially non-adhesive rubber such as the film or coating of coalesced rubber particles deposited from a dried coating of unvulcanized natural rubber latex. While other known cohesive, substantially non-adhesive materials may

2

be used as the self-adherent coating for the wrapping paper of the present invention, such as unvulcanized Buna S latex, the latices of other unvulcanized synthetic rubbers, and the plasticized polyvinyl acetate compositions disclosed in Patent No. 2,371,001, granted March 6, 1945, or any mixture of such materials including natural rubber, the coating of unvulcanized natural rubber deposited from a latex of the same is preferred because such a coating cooperates uniformly effectively with the wax film in imparting the property of moisture-proofness or moisture-vapor-proofness to the paper sheet.

Any paper-thin, flexible carrier sheet which 15 lends itself for use in wrapping small articles may be used in accordance with my invention, although paper is preferred as noted above. With such sheets, the rubber (natural and/or synthetic) or other cohesive, substantially non-adhesive material cooperates with the wax to seal any imperfections in the sheet and/or to impart the desired moisture-proof or moisture-vapor-proof properties to the sheet. When paper is used as the carrier sheet it is preferred that it 20 be a lightly sized paper which permits some surface penetration of latex (natural or synthetic rubber). Other papers such as hard sized papers may, of course, be used. With such hard sized papers it may be necessary to overcome the effect 25 of this sizing by the addition to the latex of a surface active agent to reduce the surface tension of the latex and to increase the wetting and penetrating power thereof. Any suitable surface active agent may be used for this purpose. Examples 30 of suitable surface active agents are sodium lauryl sulphate, sodium cetyl sulphate, the sodium salt of the dioctyl ester of sulfosuccinic acid (Aerosol OT), the sodium sulphate derivatives of 7-ethyl-2-methyl-undecanol-4 (Tergitol 4) and 3,9-diethyl tridecanol-6 (Tergitol 7), decyl benzene sodium sulfonate (Santomerse 5), and phenyl-para-toluene sulfonate.

A suitable cohesive, substantially non-adhesive film in accordance with the preferred 45 aspects of the present invention may be formed by applying to the paper sheet a coating of a conventional, commercially available, ammonia-stabilized, unvulcanized natural rubber latex, and drying the same. This latex may or may not contain an anti-oxidant for the rubber, as desired. The film of rubber deposited from this latex inherently has the desired cohesive, substantially non-adhesive properties.

Desired cohesive, substantially non-adhesive 55 properties of a film deposited from a latex of un-

vulcanized natural rubber may be obtained by compounding the latex with controlled amounts of a water-soluble colloid which is compatible with the latex and which serves to destroy adhesiveness and tackiness in the dried latex, and a small amount of a water-soluble, comparatively non-volatile plasticizer, as described in Patent No. 2,000,763, granted May 7, 1935. A typical latex composition as given in this patent is made by mixing a commercial unvulcanized natural rubber latex of about a 35% solid content with about 25% by volume of a stiff tapioca starch paste or a water-soluble casein paste, and about 2% to 5% by volume of glycerine.

As pointed out above, any cohesive, substantially non-adhesive material may be used in accordance with the present invention. Thus, such materials may be made or compounded in accordance with known procedures from aqueous dispersions or latices of diolefin polymers other than natural rubber, such as gutta percha, balata, polyisoprenes and the like; or from synthetic rubbers such as butadiene polymers, for example, buna rubber, butylene polymers such as polyisobutylene (Vistanex) and butadiene copolymers such as the co-polymers of butadiene and styrene (Buna S, Hycar OS, etc.) and butadiene and acrylonitrile (Buna N, Hycar OR, Thiokol RD, etc.); Buna S and Buna N "cold" rubbers which are obtained by copolymerization at temperatures below normal room temperatures and preferably at temperatures of about 41° F. and below; chloroprenes such as chloroprene alone or co-polymerized with acrylonitrile, etc. (Neoprene); co-polymers of olefins and diolefins such as isobutylene and butadiene or isoprene (Sutyl rubber); organic polysulfides such as ethylene polysulfide formed by reacting ethylene dichloride and sodium tetrasulfide (Thiokol A); the reaction product of  $\beta, \beta'$ -dichloroethyl ether and sodium tetrasulfide (Thiokol B or Perduren G); and rubbers derived from unsaturated long-chain acids from soybean and other oils polymerized and then esterified with a glycol such as ethylene glycol (Norepol, Agripol).

Other synthetic rubber latices may be used to make the cohesive, substantially non-adhesive materials used in accordance with my invention and these may be any latex selected from the class prepared by the polymerization in aqueous emulsion of a butadiene-1,3 hydrocarbon such as butadiene-1,3, isoprene, 2,3-dimethyl butadiene-1,3, piperylene or the like either alone or in admixture with each other and/or in admixture with lesser or equal amounts of one or more monoethylenic compounds copolymerizable therewith in aqueous emulsion such as acrylonitrile, methacrylonitrile, alpha-chloro acrylonitrile and similar acrylic nitriles; styrene, vinyl naphthalene, p-chloro-styrene and similar aryl olefins and substituted aryl olefins; methyl acrylate, methyl methacrylate, acrylamide and similar esters and amides of acrylic acids; methyl isopropenyl ketone, vinylidene chloride, isobutylene, methylvinyl ether, and other compounds containing a single ethylenic double bond,  $>C=C<$ , which are copolymerizable with butadiene-1,3 hydrocarbons in aqueous emulsion. In fact, any of the compounds which may be termed butalastics as defined in the book "Butalastic Polymers, A Treatise on Synthetic Rubbers" by Marchionna may be used.

The cohesive, substantially non-adhesive materials may be formed from synthetic resins other than those described in the above noted Patent

No. 2,371,001. Thus they may be formed from co-polymers of polyvinyl acetate and polyvinyl chloride, polyvinyl acrylate, polyvinyl methacrylate, polyvinyl ethacrylate and like acrylates having from 1 to 5 carbon atoms in the alkyl group, polyvinyl ethers, polyvinyl ketones such as methyl vinyl ketone, polyvinyl alcohol, polyvinyl acetals such as formal, butyral, etc., and the like.

- 10 As is manifest from the foregoing, any rubber, synthetic rubber and synthetic resin, or any mixture thereof, may be used in forming the cohesive, substantially non-adhesive materials used in accordance with the present invention. In 15 general the rubbers and resins are used in aqueous dispersion (lattice) form. The amount of cohesive material applied to the carrier sheet may be varied widely, say from about 0.2 lb. to 2 lbs. (solids) per 144 sq. yds. of carrier sheet.
- 20 The following are examples of cohesive, substantially non-adhesive materials including such latices.

|                                                        | Parts by weight |
|--------------------------------------------------------|-----------------|
| 1. Natural rubber latex                                | 100.0           |
| 25 Dibutanaphthyl p-phenylene diamine<br>(antioxidant) | 1.0             |
| 2. Butadiene-styrene copolymer                         | 100.0           |
| Sodium silicate                                        | 0.5             |
| Antioxidant as in Example 1                            | 1.0             |
| 30 Ester gum                                           | 1.0             |
| 3. Butadiene-acrylonitrile                             | 100.0           |
| Sodium silicate                                        | 0.5             |
| Antioxidant as in Example 1                            | 1.0             |
| Ester gum                                              | 1.0             |
| 35 4. Polyvinyl acrylate latex                         | 100.00          |
| Antioxidant as in Example 1                            | 1.0             |
| 5. Chloroprene                                         | 100.0           |
| Sodium cetyl sulphate                                  | 0.5             |
| Antioxidant as in Example 1                            | 1.0             |
| 40 Zinc oxide                                          | 5.0             |
| Ester gum                                              | 1.0             |

- Any suitable wax or wax-like material such as paraffin wax, beeswax, montan wax, carnauba wax, synthetic waxes such as the high melting point synthetic wax sold by Glyco Products Co., Inc., under the trade-mark Acrawax C, and the like may be used as the moisture-proof coating for the wrapping material of the present invention. This coating may be applied to the carrier sheet in any desirable manner, in aqueous emulsion form from solvent solution, or from molten bath, for example, as is well understood. Other suitable moisture-proof materials such as the known plastic compositions of wax and rubber 55 may also be used, as may also the relatively high melting point microcrystalline waxes. When such waxes are combined with the cohesive, substantially non-adhesive materials on opposite sides of a paper carrier sheet, the carrier sheet is rendered moisture-vapor-proof. As is known, such waxes consist of amorphous, substantially saturated compounds that have been formed from high boiling point, non-saturated petroleum derivatives by way of polymerization and possibly by condensation (which products in the raw state are known commercially as petroatum); and, more specifically, those higher melting point substances separated therefrom and sold as petroleum wax. These microcrystalline waxes may be used alone or they may be admixed with a material such as coumarone resin, phenol-formaldehyde resin, copal gum and the like, which will form a colloidal suspension or 65 gel with the microcrystalline wax, to increase 70 the cohesive, substantially non-adhesive properties of the carrier sheet.

the inherent adhesiveness of the wax, as described in the Dreymann Patent No. 2,031,036.

The present invention will be fully understood from the foregoing and from the following description of a preferred illustrative embodiment of the invention and of some uses thereof, as illustrated in the accompanying drawings, wherein:

Figure 1 is a perspective view of a coated sheet of paper embodying the present invention;

Fig. 2 is an enlarged cross-sectional view thereof taken along the line 2—2 of Fig. 1;

Fig. 3 illustrates the use of the coated paper of Fig. 1 for wrapping a sandwich, the latter being shown as resting on the cohesive surface of the paper;

Fig. 4 is a cross-sectional view of the wrapped sandwich taken substantially along the line 4—4 of Fig. 3;

Fig. 5 is a similar cross-sectional view taken substantially along the line 5—5 of Fig. 4;

Fig. 6 illustrates the use of the paper of Fig. 1 for wrapping foodstuffs which are contained in an article such as a dish;

Fig. 7 depicts the package formed by wrapping the paper about the foodstuffs in the dish in accordance with the present invention; and

Figs. 8 and 9 illustrate modified embodiments of the coated sheets of the present invention.

In the drawings the numeral 10 designates a flexible paper sheet, preferably a lightly sized paper sheet which permits of some surface penetration of a latex, the numeral 11 designates a wax or other water-proof or moisture-vapor-proof coating, and the numeral 12 designates the cohesive, substantially nonadhesive coating, preferably of natural rubber latex and preferably applied uniformly and lightly over the surface of the paper. As pointed out above, the preferred cohesive, substantially nonadhesive coating is formed by drying an unvulcanized natural latex upon the surface of a sheet of paper. The solids content of this or any other latex which may be used in accordance with the present invention may be varied widely, as desired, from about 10% to about 50% to 60%. For most purposes about a 35% solids content latex is suitable.

In the use of this coated paper to wrap comestibles, for example, a sandwich, the sandwich, indicated by the numeral 15, is placed upon the cohesive coating of the paper sheet adjacent one end and within the boundaries thereof, as illustrated in Fig. 3. The other end of the coated sheet is then folded over the sandwich so that marginal portions of the cohesive coating of the folded sheet are in opposed relationship. A light pressure is then applied to the opposed surfaces of the cohesive coating by running the fingers lightly around the marginal portions of the folded paper, thereby completely sealing the sandwich within a moisture-proof package, illustrated in Figs. 4 and 5.

In the use of the paper of the present invention to wrap foodstuff contained within a dish or other article, the article containing the foodstuff, indicated by the numeral 17, is placed upon the cohesive coating of the paper, as shown in Fig. 6, and the free ends of the paper are pulled up around the foodstuff and bunched together with the cohesive coating surfaces in opposing relationship, thereby enclosing the foodstuff in a water-proof package which may be placed in a refrigerator until ready for use.

Due to the moisture-proof or moisture-vapor-

proof characteristics of the wrapping sheet of the present invention, foodstuffs wrapped within this sheet may be kept within a refrigerator for substantial periods of time, without desiccation or decay and without acquiring the flavors of other foodstuffs. The contents of the package may be readily removed either by cutting the wrapper or by pulling it apart at the joining surfaces. In the latter case, if care is exercised in pulling the surfaces apart, the sheet may be re-used.

The coated paper sheet referred to above has the cohesive, substantially non-adhesive coating all over one surface thereof and the wax over the other surface and these sheets may be stacked one upon the other without adherence, by placing the cohesive coating of one sheet in contact with the wax coating of another.

The versatility of the coated sheet to wrap various articles may be increased by applying additional zones of the cohesive, substantially non-adhesive coating on the side of the sheet containing the wax or other water-proof coating, as illustrated in Figs. 8 and 9. In making these sheets the paper or other carrier sheet is coated on one side throughout the area thereof with a cohesive, substantially non-adhesive coating as before and a similar coating is applied to the margins or other desired portions of the opposite side. The wax is then applied to the carrier sheet between the areas delineated by the zones of cohesive, substantially non-adhesive coating.

In Fig. 9, the cohesive, substantially non-adhesive coating 18 is applied all over the surface of one side of the carrier sheet and, additionally, along the longitudinal margins 19 on the opposite sides. The wax coating 20 is applied to the carrier sheet over the area between the zones of cohesive, substantially non-adhesive coating. In the embodiment of the invention illustrated in Fig. 8, there are additional zones of cohesive, substantially non-adhesive coating 21 which extend between the marginal zones 19 of cohesive, substantially nonadhesive coating, at intervals throughout the length of the sheet.

For convenience of the user any of the coated sheets described above may be vended in the form of a roll, illustrated in Fig. 8, and transverse perforations of score lines, illustrated by the score lines 22, may be provided to enable the user to tear a piece of this wrapping sheet from the roll. Where the wrapping sheet of the present invention is provided with cohesive, substantially non-adhesive coatings on both sides, as in Figs. 8 and 9, stacked individual sheets may be interleaved with Holland cloth or other liner material, or the coated wrapping sheet may be wound on the roll with a liner material (not shown) to prevent the opposed cohesive surfaces from adhering to one another, as is well understood.

The term "a rubber" is employed in the claims to define a vulcanizable or non-vulcanizable plastic material which possesses high extensibility under load coupled with the property of forcibly retracting to approximately its original size and shape after the load is removed. Such materials include for example, gutta percha, balata, copolymers of butadiene with styrene and acrylonitrile, etc., as pointed out above.

70 I claim:

1. As a new article of manufacture, a sheet of self-sealing wrapping paper comprising a flexible paper base having a cohesive, substantially dry, non-adhesive and non-tacky wax-free coating consisting essentially of unvulcanized

75

natural rubber on the entire area of one side thereof and marginal zones of a similar coating on its other side, said other side of the paper base having an exposed comparatively thin flexible film of wax over the area between said zones, said coatings being exposed and adapted, when portions thereof are brought into engagement with one another by slight pressure during a wrapping operation, to have such portions adhere to one another by cohesion, and serving to assist the wax film in rendering the sheet moisture-proof.

2. As a new article of manufacture, a sheet of self-sealing wrapping paper comprising a thin flexible calendered paper base having a cohesive, substantially dry, non-adhesive and non-tacky wax-free coating consisting essentially of unvulcanized natural rubber on the entire area of one side thereof and zones of a similar coating on its other side, said other side of the paper base having an exposed flexible film of wax over the area between said zones, said coatings being exposed and adapted, when portions thereof are brought into engagement with one another by slight pressure during a wrapping operation, to have such portions adhere to one another by cohesion, and serving to assist the wax film in rendering the sheet moisture-proof.

3. As a new article of manufacture, a sheet of self-sealing wrapping material comprising a thin fibrous film base having on the entire area of one side thereof only an exposed comparatively thin flexible wax coating for purposes of moisture-proofing the sheet and on the entire area of its other side an exposed wax-free coating consisting essentially of unvulcanized natural rubber deposited from an aqueous latex dispersion containing a small amount of material selected from the group consisting of starches and caseins, said last mentioned coating being cohesive, substantially dry, non-adhesive and non-tacky and adapted, when portions thereof are brought into engagement with one another by slight pressure during a wrapping operation to have such portions adhere to each other by cohesion, and serving to assist the wax coating in rendering the sheet moisture-proof.

4. As a new article of manufacture, a sheet of self-sealing wrapping paper comprising a thin flexible paper base having on the entire area of one side thereof only an exposed comparatively thin flexible wax coating for purposes of moisture-proofing the sheet and on the entire area of its other side an exposed wax-free coating consisting essentially of unvulcanized natural rubber deposited from an aqueous latex dispersion containing a small amount of material selected from the group consisting of starches and caseins, and in addition a hydroscopic substance, said last mentioned coating being cohesive, substantially dry, non-adhesive and non-tacky and adapted to stick only to itself and, when portions thereof are brought into engagement with one another by slight pressure during a wrapping operation to have such portions adhere to each other by cohesion, and serving to assist the wax coating in rendering the sheet moisture-proof.

5. As a new article of manufacture, a moisture-proof sheet of self-sealing wrapping material adapted completely to encase an article and thereby seal the same against outside moisture, said article comprising a thin flexible paper sheet normally pervious to moisture, said sheet having on one surface thereof an exposed comparatively thin flexible wax film coating completely covering said surface and thereby imparting moisture-

proof properties thereto and on its other surface an exposed flexible dried wax-free film consisting essentially of coalesced unvulcanized natural rubber particles, said film covering the complete said other surface of the sheet and being substantially dry and non-tacky and yieldingly self-adhering when portions thereof are brought into engagement, but being non-adhesive to such surfaces as wood, glass and metal, the said non-tacky self-adhering film cooperating with said wax coating in moisture-proofing said paper sheet.

6. As a new article of manufacture, a moisture-proof sheet of self-sealing wrapping material adapted completely to encase an article and thereby seal the same against outside moisture, said article comprising a thin flexible paper sheet normally pervious to moisture, said sheet having on one surface thereof an exposed comparatively thin flexible wax film coating completely covering said surface and thereby imparting moisture-proof properties thereto and on its other surface an exposed flexible dried wax-free film consisting essentially of coalesced unvulcanized rubber particles, said last mentioned film covering the complete said other surface of the sheet and being substantially dry and non-tacky and yieldingly self-adhering when portions thereof are brought into engagement, but being non-adhesive to such surfaces as wood, glass and metal, the said non-tacky self-adhering film cooperating with said wax coating in moisture-proofing said paper sheet.

7. As a new article of manufacture, a moisture-proof sheet of self-sealing wrapping material adapted completely to encase an article and thereby seal the same against outside moisture, said article comprising a thin flexible paper sheet normally pervious to moisture, said sheet having on one surface thereof an exposed comparatively thin flexible wax film coating completely covering said surface and thereby imparting moisture-proof properties thereto and on its other surface an exposed flexible dried wax-free film consisting essentially of a rubber in an unvulcanized state, said last mentioned film covering the complete said other surface of the sheet and being substantially dry and non-tacky and yieldingly self-adhering when portions thereof are brought into engagement, but being non-adhesive to such surfaces as wood, glass, and metal, the said non-tacky self-adhering film cooperating with said wax coating in moisture-proofing said paper sheet.

8. As a new article of manufacture, a sheet of self-sealing wrapping paper comprising a flexible paper base having a cohesive, substantially dry, non-adhesive and non-tacky wax-free coating consisting essentially of a rubber in an unvulcanized state on the entire area of one side thereof and marginal zones of a similar coating on its other side, said other side of the paper base having an exposed comparatively thin flexible film of wax over the area between said zones, said coatings being exposed and adapted, when portions thereof are brought into engagement with one another by slight pressure during a wrapping operation, to have such portions adhere to one another by cohesion, and serving to assist the wax film in rendering the sheet moisture-proof.

9. As a new article of manufacture, a sheet of self-sealing wrapping paper comprising a thin flexible calendered paper base having a cohesive, substantially dry, non-adhesive and non-tacky wax-free coating consisting essentially of a rubber in an unvulcanized state on the entire area

of one side thereof and zones of a similar coating on its other side, said other side of the paper base having an exposed flexible film of wax over the area between said zones, said coatings being exposed and adapted, when portions thereof are brought into engagement with one another by slight pressure during a wrapping operation, to have such portions adhere to one another by cohesion, and serving to assist the wax film in rendering the sheet moisture-proof.

BERTRAM L. TRILICH.

**REFERENCES CITED**

The following references are of record in the file of this patent:

10  
15

**UNITED STATES PATENTS**

| Number      | Name          | Date           |
|-------------|---------------|----------------|
| 1,723,581   | Ruderman      | Aug. 6, 1929   |
| 2,118,101   | Nollan et al. | May 24, 1938   |
| 5 2,173,989 | Wilbur        | Sept. 26, 1939 |
| 2,224,189   | Leslie        | Dec. 10, 1940  |
| 2,354,060   | Rhodes et al. | July 18, 1944  |
| 2,439,481   | Martin        | Apr. 13, 1948  |

**FOREIGN PATENTS**

| Number  | Country       | Date          |
|---------|---------------|---------------|
| 365,466 | Great Britain | Jan. 21, 1932 |